

(Model.)

H. M. KITCHELL.

DIE FOR EMBOSSED PAPER AND LIKE IMPRESSIBLE MATERIALS.

No. 440,166.

Patented Nov. 11, 1890.



Witnesses

H. J. Williams  
J. L. Steiner

Inventor

Hudson M. Kitchell  
By his Attorney  
W. L. Remond

# UNITED STATES PATENT OFFICE.

HUDSON M. KITCHELL, OF BROOKLYN, NEW YORK.

## DIE FOR EMBOSSED PAPER AND LIKE IMPRESSIBLE MATERIALS.

SPECIFICATION forming part of Letters Patent No. 440,166, dated November 11, 1890.

Application filed April 12, 1890. Serial No. 347,733. (Model.)

*To all whom it may concern:*

Be it known that I, HUDSON M. KITCHELL, a citizen of the United States, residing at Brooklyn, in the county of Kings and State 5 of New York, have invented and made certain Improvements in Dies for Embossing Paper and Like Impressible Materials; and I hereby declare that the following specification is a full, clear, and exact description and explanation of the same, so that those skilled 10 in the art of embossing impressible materials may understand and use the same, reference being had to the accompanying drawing in which—

- 15 A is the die.  
B is the cardboard.  
C is the plastic composition.

I am aware that paper and other materials of like impressionable character have heretofore 20 been embossed by means of dies with various raised or depressed designs, such dies having been made from some metal with the designs engraved in it or electrotyped upon it.

I am also aware that molds have been made 25 of soft plastic materials and compositions of materials for molding metals; but I am not aware that previous to my discovery and invention thereof dies have ever been made of soft plastic material with a hard flat flexible back, and while the engraved surface is 30 soft designs can be cut or engraved in it, and then hardened to such a point that the material from which the dies are made will be both hard to resist abrasion and tough enough to 35 resist cracking while being passed between rolls in embossing pliable materials.

The ingredients composing the plastic compound are as follows: glue, molasses, water, and plaster-of-paris in the following proportions: dissolved glue, one pound; water, one 40 gallon; molasses, one pint; plaster-of-paris, twenty pounds. These ingredients are then placed in a receptacle and thoroughly mixed together. It then becomes a thick sticky 45 mass that can be easily worked.

The *modus operandi* employed in making the die A is as follows: The composition after being mixed is poured on a large sheet of hard flat flexible material—such as cardboard B—and worked over the surface of the 50 card-board with the hands or a brush until it is perfectly smooth and of an even thickness all over the surface. The design is then engraved in the plastic composition C while it is still in a wet state. The implements used 55 in engraving the designs are small pieces of wood with their points sharpened to various thicknesses. The die is then allowed to dry, and when thoroughly dry is ready for use.

What I claim, and desire to secure by Letters Patent, is—

The herein-described hard flat flexible die, the body of which is a hard flat flexible material, such as card-board, and the engraved surface of which is formed of a hardened 65 plastic material, whereby it may be passed between rolls without cracking, substantially as set forth.

HUDSON M. KITCHELL.

Witnesses:

JAMES M. HICKS,  
W. L. BENNEM.